

No. 785,002.

PATENTED MAR. 14, 1905.

J. J. HUDSON.

MANUFACTURE OF IRON AND STEEL.

APPLICATION FILED MAR. 9, 1904.



*WITNESSES:*

John H. Buek.

Wesley H. Ruel.

*INVENTOR:*

James Jones Hudson

by his Attorneys,

Hudson & Hudson

## UNITED STATES PATENT OFFICE.

JAMES JONES HUDSON, OF PHILADELPHIA, PENNSYLVANIA.

## MANUFACTURE OF IRON AND STEEL.

SPECIFICATION forming part of Letters Patent No. 785,002, dated March 14, 1905.

Application filed March 9, 1904. Serial No. 197,212.

*To all whom it may concern:*

Be it known that I, JAMES JONES HUDSON, a citizen of the United States, residing in Philadelphia, Pennsylvania, have invented certain 5 Improvements in the Manufacture of Iron and Steel, of which the following is a specification.

My invention relates to the manufacture of what is familiarly known as "charcoal-iron"— 10 that is to say, iron melted in the presence of charcoal, which may or may not be employed as the heating and melting medium.

In carrying my invention into effect I melt the metal in the presence of charcoal in a 15 suitable furnace heated by means of oil, gas, or hydrocarbon vapor and maintain it in a molten condition, at the same time introducing blasts of air to the molten metal for the purpose of boiling it, which method of procedure 20 has the effect of refining such iron by decarbonization and oxidation, the metal filtering through the charcoal and the latter consuming the impurities as they are eliminated from the molten mass. In some instances I may 25 add some charcoal to the metal after it has reached a molten condition to insure the combustion and dissipation of any injurious gases arising during the boiling operation.

My improved process of manufacturing 30 charcoal-iron may be applied to the manufacture of charcoal-steel with equally-valuable results.

The process forming the subject of my invention may be carried out in furnaces of different character, and as illustrating one type 35 of furnace capable of carrying my invention into effect reference is had to the accompanying drawings, in which—

Figure 1 is a sectional plan view of said furnace. Fig. 2 is a longitudinal sectional view on the line *a a*, Fig. 1. Fig. 3 is a cross-sectional view on the line *b b*, Fig. 2; and Figs. 4 and 5 are views of an adjustable twyer.

In the old or common process of manufacturing charcoal-iron the method of procedure 45 is as follows: Metal from a run-out fire, scrap, or other suitable or convenient material to the amount of two hundred and fifty to three hundred pounds, together with charcoal, is

thrown at one charge into an open, nobbling, 50 or sinking fire, and in this fire it is formed into what is variously known as a "masse," "bloom," "lump," or "loupe," hereinafter referred to as a "loupe." As the metal melts it falls to the bottom of the furnace and cools, 55 and in leaving the heated zone of the furnace it frequently carries portions of raw or unmelted iron with it. In order to melt this raw addition to the metal, the forgeman is obliged to raise the mass with a suitable bar, 60 so as to bring it back to the highly-heated part of the furnace. This requirement, as may be readily understood, is laborious, uncertain, and costly, and it is impossible to produce a perfect homogeneous metal of standard grade. 65 The run-out fires, however, have been generally abandoned because too expensive, so that the material used for the charge is iron and steel scrap of all grades, such as are on the market to-day, and I may here state as one of 70 the primary and principal defects of the old process that the small amount of refining this material gets in sinking in the old-fashioned fire, as just explained, is not sufficient to change it to any great degree, so as to produce a pure and homogeneous iron. From the nobbling-fire the loupe is taken to the hammer to be shaped for the muck-rolls. Before going to the rolls, however, the "bloom" (as it is now called) is reheated in a heating-furnace and 75 then taken to the mill to be rolled out into what are called "charcoal" muck-bars. When cold, these bars are cut in pieces the length of which depends on the weight of pile desired, which is generally five or six barshigh. 80 These bars are again put in the heating-furnace and afterward rolled into plates, boiler-tube skelp, bars for tin-plate, or any other shape for which charcoal-iron is used.

The defects of the old process are quite numerous, some of which are as follows: As the metal sinks through the mass of fuel pieces of scrap or raw iron will sink into the softer part of the loupe without being refined, and pieces will also stick to the surface of the 85 loupe and be hammered in, a condition which will result in the iron containing flaws and blisters. One forgeman might by chance

make a fairly good loupe, while the forgeman on the next fire might make an inferior one, and when cut in pieces for the bars to pile the inferior bars will spoil the good ones. Also 5 a pile would be made up of bars of different makes—*i. e.*, of different analyses—so that there would be no uniformity of quality. In heating the bars it is necessary to have a good welding heat in order to properly weld them, 10 for if not properly welded they will show up in flaws and blisters. On the other hand, if the heater produces too high a heat, which he is apt to do, and burns such bars the nature of the iron is destroyed. Another defect 15 which very often occurs is that occasioned by some unavoidable delay in taking the loupe from the fire, causing carburization. These objections all tend to lead to the abandonment of weldable iron, as by the old process 20 it is impossible to obtain a pure and homogeneous metal. According to my improved process, however, which I will now proceed to describe, I do away with the preliminary forging and shaping of the mass of metal and 25 run the molten metal, after it has been refined and brought to the proper analysis, directly into a suitable mold, from which it may be taken as soon as it has received a surface chill, given a wash heat in a suitable furnace or oven, and then passed directly to the mills to be rolled into skelp, plates, or other suitable shapes.

The mixture for a high grade of charcoal-iron made in accordance with my invention 35 may be as follows, supposing it is desired to make fifteen tons: iron ore, one ton; cast and pig iron, six tons; wrought-iron and steel scrap, eight tons. For this amount of metal about fifteen bushels of charcoal per ton of 40 other material will be required.

In carrying out my improved process I may use any suitable form of furnace, and in the present instance I have shown a simple form of melting-furnace capable of carrying 45 out my improved process.

In the drawings the furnace-body is shown at 1 with feed-openings 2, a tap-hole 3, closed by a plug 4, and twyer-openings 5, in which are mounted the tuyers 6. At the ends of 50 the furnace the pipes 10 are provided, which discharge gas, oil, or a suitable hydrocarbon vapor that is ignited and serves to heat the furnace. The bed of the furnace is indicated at 11, and the layers of charcoal and metal 55 are shown in the preferred method of charging the furnace, being indicated at 12 and 13, respectively, Figs. 2 and 3. In Figs. 1 and 3 the feed-openings are shown closed by doors 14, and the furnace is supposed to be in condition to melt the metal. During this action 60 the products of combustion will pass out through the end opening 15 to any suitable discharge-outlet. After the metal is melted, maintained in the molten condition, and re- 65 fined to the proper degree the plug 4 may be

removed, and the metal will run out of the tap-opening 3 to any suitable mold or other receptacle.

A form of adjustable twyer for use with the melting-furnace I have shown for carrying out my invention is fully illustrated in Figs. 4 and 5. The twyer-opening 5 is in the form of a conical recess with its smallest end opening into the melting-chamber. The twyer 6 is adjustable up and down in this recess by 70 the following means: Extending rearwardly from the bottom of the twyer is a projection 20, which is connected to a stirrup 21, hung from a threaded stem 22. Carried by the side of the furnace is a supporting-bracket 23, 75 carrying a threaded bolt 24, and a turnbuckle 25 is used for connecting these threaded members. By operating this turnbuckle the stirrup may be raised and lowered, and with it the twyer. To guide the twyer in its vertical movement, I provide the side plates 26, which are slotted at 27 to receive the ends of a bolt or bar 28, carried by the stirrup. This slot is curved in the arc of a circle struck from the point of contact of the twyer with 80 the inner wall of the furnace. A blast-pipe 30 is connected to the twyer by means of a flexible section 31, which may be of leather or any suitable substance commonly used for the purpose, and the water-pipes 32, two in 85 number, are also connected to the twyer by means of flexible sections 33. These flexible sections provide for ready connection of these members and at the same time permit a wide range of adjustment for the twyer.

The furnace, of whatever design employed, is charged with the scrap, pig-iron, and ore to the amount of fifteen tons, with the proper addition of charcoal, and the tuyers, which are preferably adjustably mounted, as just described, or other means of discharging air under pressure to the charge are set so as to deliver the air-blast through the mass of material. Before charging the furnace, however, it is preferably brought to a proper heat by 100 any suitable means—by preference gas, hydrocarbon vapor, or oil discharging from the pipes 10, (although in some instances I may use coal)—and then the charge is inserted and melted and kept in a molten condition, charcoal being added to increase the heat and continue the refining. While in this molten condition it will be boiled and thoroughly refined by means of the charcoal, air-blast, and other source of heat, eliminating sulfur, phosphorus, silicon, and other injurious ingredients to an extent hitherto unknown in the manufacture of iron and steel, the mass being 105 decarburized until the analysis of the molten metal which may be made from time to time 115 shows the quality of iron required, thereby enabling me to produce any desired uniform grade of charcoal iron or steel. The resultant metal will be found to be of superior quality 120 and of the greatest value in the manufacture 125 130

of boiler tubes and plates, and as soon as its analysis shows the quality desired it is drawn from the furnace into masses of different shape and size, according to the kind of iron 5 to be rolled, and after it has received a surface chill it is given a wash heat in a suitable furnace or oven and may then be passed directly to the mill, where it is rolled into plates, skelp, or bars for tin-plate or any other suitable shapes.

For a cheap grade of charcoal-iron I may increase the quantity of iron ore and cast-scrap and pig-iron and besides reducing the quantity of wrought and steel scrap I may, 15 use a cheaper grade of scrap and add only about twelve bushels of charcoal to each ton of the mixture. While I prefer to use cold air for the blast in most instances in producing the cheaper metal, I may employ a blast 20 of heated air, as this enables me to use a less amount of the charcoal fuel.

My improved process of using charcoal in the manufacture of charcoal-iron may also be used to advantage in the manufacture of steel. 25 Mild steel is at present used because of its relative cheapness for many purposes for which charcoal-iron should be used. I propose to refine such steel by the use of charcoal, and thereby render it available for all 30 purposes for which charcoal-iron of the best grade is available. I may do this in a furnace similar to the one shown for carrying out my improved charcoal-iron process, although it will be understood that I may use 35 any suitable form of melting-furnace having provision for heating the same by oil, gas, or hydrocarbon fuel and for introducing air in blasts through suitable twyvers, preferably adjustably mounted. After thoroughly re- 40 fining the mass by means of the charcoal, eliminating the injurious elements, I recarbonize it with accuracy and produce a pure and high-grade steel.

For a mixture of fifteen tons of steel I may 45 use the following proportions: wrought-iron and steel scrap, nine tons; pig-iron, six tons. For this amount of metal about fifteen bushels of charcoal per ton will be required. After the metal is melted its subsequent treatment 50 may be similar to the treatment of the charcoal-iron just described.

The advantages of my improved process of manufacturing charcoal iron and steel are as follows: The resultant metal contains no 55 pieces of scrap or raw iron sunk into the same unrefined. Hence I produce a perfect iron and steel of higher grade than that which is produced by the old process. I do away with the preliminary forging and shaping of 60 the mass of metal and rolling the same into muck-bars. In the old process too much depends on chance, because there is no way of taking an analysis, and even with conscientious care and effort on the part of the work- 65 men they cannot prevent defects in the iron

or insure a homogeneous product, while with the improved process forming the subject of my invention charcoal-iron or charcoal-steel can be produced with any analysis the trade may require. Besides producing a homogeneous iron and steel and of a high grade another advantage of my process is a considerable reduction of cost, making it possible to put on the market metal that is reliable at a price that will encourage its use for purposes where the 70 superiority of charcoal-iron is unquestioned. While the melting of iron or steel and the continuance of such metal in a molten condition will refine it to a certain extent, there are certain impurities that will not respond to 80 this treatment to a degree sufficient to produce a metal of high grade. With the use of charcoal, however, the molten metal in passing through it leaves behind its impurities, which are consumed by the charcoal, the latter having a certain affinity for this action not obtainable when the metal is melted and boiled in the ordinary manner.

Having thus described my invention, I claim and desire to secure by Letters Patent— 90

1. The improvement in the art of manufacturing iron and steel, which consists in placing a combined charge of charcoal and the material to form such metal upon the hearth or bottom of a furnace, melting said metal with the 95 charcoal, and maintaining a molten bath of the metal in contact with the charcoal until the completion of the heat.

2. The improvement in the art of manufacturing iron and steel, which consists in placing a combined charge of charcoal and the material to form such metal upon the hearth or bottom of a furnace, heating said furnace to a temperature sufficient to melt said metal with the charcoal, and maintaining a molten bath 105 of the metal in contact with the charcoal until the completion of the heat.

3. The improvement in the art of manufacturing iron and steel, which consists in placing a charge of charcoal upon the hearth or bottom 110 of a furnace, placing material to form such metal upon said charcoal, melting said metal with the charcoal, and maintaining a molten bath of the metal in contact with the charcoal until the completion of the heat. 115

4. The improvement in the art of manufacturing iron and steel, which consists in heating a suitable furnace, placing a charge of charcoal upon the hearth or bottom of the same, placing the material to form such metal 120 upon said charcoal, introducing a blast of air to raise the heat of the furnace and melt the metal, and then maintaining said metal in a molten bath in contact with the charcoal until the completion of the heat.

5. The improvement in the art of manufacturing iron and steel, which consists in heating a suitable furnace, placing a charge of charcoal upon the hearth or bottom of the same, placing a charge of iron upon said char- 130

coal, introducing a blast of air to raise the temperature sufficiently to melt and refine said charge, and maintaining a molten bath of the metal in contact with the charcoal until the completion of the heat.

6. The improvement in the art of manufacturing iron and steel, which consists in heating a suitable furnace, placing a charge of charcoal and iron upon the hearth or bottom of the same, introducing a blast of air to increase the heat and melt said charge, and then maintaining a molten bath of the metal in contact with the charcoal until the completion of the heat.

15 7. The improvement in the art of manufacturing iron and steel, which consists in heating a suitable furnace, placing a charge of charcoal and iron upon the bottom or hearth of the same, introducing a blast of air to increase the heat and effect the melting of the charge, and maintaining said blast until the iron is caused to boil in the presence of the charcoal whereby it may be refined by the charcoal and maintained in a molten condition 25 in contact therewith until the completion of the heat.

8. The improvement in the art of manufacturing charcoal iron and steel of uniform grade or quality, which consists in heating a suitable furnace, placing a charge of charcoal and iron upon the hearth or bottom of the same, introducing a blast of air to increase the heat of the furnace and thereby melt the metal, maintaining such metal in a molten condition in 30 the presence of the charcoal whereby it may be refined by the same until the metal shows the analysis desired, such process being carried on in such a manner as to permit testing and analysis of the metal from time to time, 35 and then casting said metal substantially as described.

9. The improvement in the art of manufacturing charcoal iron and steel, which consists in heating a suitable furnace, charging the same with alternate layers of charcoal and iron, introducing a blast of air to assist the combustion and raise the melting heat, and 40

50 maintaining a molten bath of the metal in contact with the charcoal until the impurities of the metal are burned out and the heat has been completed.

10. The improvement in the art of manufacturing charcoal iron and steel, which consists in heating a suitable furnace, charging the same with alternate layers of charcoal and iron, introducing a blast of air to assist the combustion and raise the melting heat, maintaining said metal in a molten condition in contact with the charcoal, and finally boiling it until the impurities of the metal are burned 60 out and the heat has been completed.

11. The improvement in the art of manufacturing charcoal iron and steel, which consists in heating a suitable furnace, charging the same with alternate layers of charcoal and iron, introducing a blast of air to assist the combustion and raise the melting heat, maintaining said metal in a molten condition until the impurities of the metal are burned out by the charcoal, causing said molten metal to 70 boil, and then adding a suitable fuel to the metal to burn off the gases arising during the boiling operation until the metal shows the analysis desired.

12. The improvement in the art of manufacturing iron and steel, which consists in heating a suitable furnace, placing a charge of charcoal and iron upon the hearth or bottom of the same, melting said metal, introducing a blast of air to increase the heat and cause said 80 charge to boil thereby refining the metal with the charcoal, and then finishing the boiling to bring the metal to the analysis required by the means for heating the furnace such as the gas, hydrocarbon vapor, or oil fuel, substantially as described.

In testimony whereof I have signed my name to this specification in the presence of two subscribing witnesses.

J. JONES HUDSON.

Witnesses:

MURRAY C. BOYER,  
Jos. H. KLEIN.